# EUROPEAN PATENT SPECIFICATION

(11) **EP 0 560 870 B1**
(45) Date of publication and mention of the grant of the patent: **20.03.1996**
(21) Application number: 92900967.8
(22) Date of filing: 05.12.1991
(51) Int. Cl.: B27M 3/04, B27M 3/06, B27K 5/00, B05D 7/08

(54) **PARQUET STRUCTURE AND METHOD FOR ITS MANUFACTURING**
PARKETTSTRUKTUR UND VERFAHREN ZU IHRER HERSTELLUNG
STRUCTURE DE PARQUET ET PROCEDE DE SA FABRICATION

(30) Priority: 05.12.1990 FI 906013
(43) Date of publication of application: 22.09.1993
(73) Proprietor: AHO, Jyrki, SF-02200 Espoo (FI); CASSERLY, Jutta, SF-08350 Routio (FI)
(72) Inventor: AHO, Yrjö, SF-02160 Espoo (FI)
(74) Representative: Stoffregen, Hans-Herbert, Dr. Dipl.-Phys.
(86) International application number: FI9100374
(87) International publication number: WO9210311

(56) References cited:
- EP-A- 0 440 580
- AU-A- 2 331 370
- CH-A- 440 053
- CH-A- 521 863
- DE-A- 1 492 562
- DE-A- 3 045 077
- DERWENT'S ABSTRACT No. 366 60 B/19, SU 612 944, publ. week 7919 SHITOV V S

## Description

The present invention relates to a parquet structure, wherein the direction of wood grains constituting the parquet surface layer is perpendicular or at an acute angle relative to the level of a parquet surface.

The invention relates also to a method for manufacturing a parquet, said method comprising the following operations:
- laying a parquet body with a surface layer of wood which is made of wood blocks, wherein the direction of wood grains is perpendicular or at an acute angle relative to the level of a parquet surface;
- effecting the smooth grinding of a surface and
- effecting the lacquer finish with a parquet lacquer.

The use of vertically grained wood as a surface layer offers several benefits. Wear resistance, hardness and compression strength in the direction of wood grains are clearly superior to the corresponding values in the direction perpendicular to wood grains.

However, the use of vertically grained wood as a parquet surface layer involves several problems with no satisfactory solutions, which is why no commercial breakthrough has been achieved thus far, either. One of the problems is the formation of seasoning cracks in and the after-living (dimensional variation) of vertically grained wood as a result of moisture variations. Another problem is the porosity of a finished wood surface. If a porous surface is conventionally laid with layers of parquet lacquer (e.g. UV-setting urethane lacquers), the thin lacquer film would quickly break in normal service. The film develops dot-like bursts with moisture penetrating in wood therethrough to blacken the surface. In traditional horizontal-grain parquets, use is made of a primer lacquer which is non-absorbent in wood and builds a film-like seal between wood and coating lacquer layers. The total consumption of expensive parquet lacquers remains relatively low, altogether appr. 30 - 40 g/m². However, such a parquet lacquering or varnishing technique, wherein a primer lacquer seal is applied directly to a ground wood surface, would lead in this invention to a disadvantageous and non-durable surface structure. Document DE-A-1 492 562 discloses a method for impregnating wooden products. This method, however, is not related to parquet structures.

An object of the invention is to provide a parquet structure and its manufacturing method, whereby even the otherwise good wear resistance and hardness of vertical-grain wood can yet be substantially improved while providing for an effective additional protection against the penetration of moisture and an effective binding against the forces of remaining moisture induced movements while, at the same time, the amount of an expensive parquet lacquer or varnish can be conventional.

This object is achieved by means of a parquet structure as set forth in the annexed claim 1 as well as by the application of a method as set forth in claim 8 for manufacturing a parquet.

A parquet structure of the invention will now be described in more detail with reference made to the accompanying drawings, in which
- Fig. 1: is a perspective view of a cross-sectioned parquet element having a structure of the invention.
- Fig. 2: illustrates the use of hexagonal wood blocks in the surface wood layer of a parquet.
- Fig. 3: shows a cross-section of the sandwich structure of a parquet, and
- fig. 4: is a larger-scale view showing a vertical section of the surface wood layer of a parquet with wood grains extending in vertical direction.

The manufacturing of the parquet structure of the invention proceeds as follows. A polygonal balk of fresh wood is cut perpendicularly or at an acute angle to the wood grains into blocks of suitable thickness (e.g. 14 mm thick). These wood blocks, a hexagonal example being shown in fig. 2, are impregnated with a water-soluble polyalcohol, e.g. polyethylene glycol (PEG), which is allowed to absorb and take effect in the wood blocks by replacing cell-wall water therein. Absorption can be intensified by a thermal treatment, wherein the wood blocks are heated in a microwave oven and the non-diluted, fluidization-heated PEG is applied as a film to a wood block whose internal vacuum accelerates the absorption of PEG into wood. The purpose is that the water-soluble impregnant replaces a sufficient amount of the cell-wall water in wood cells. This prevents the post-movements (dimensional variations) of wood material caused by seasoning cracks and moisture fluctuations. It is well known that the moisture-induced movements of wood result explicitly from the amount of water contained in cell walls and from the swelling and shrinking of a cell wall caused by the fluctuations thereof.

The wood blocks, thus impregnated with a water-soluble polyalcohol (e.g. PEG), are stored for 1 to 3 days at a temperature of 50 - 80^{o}C for a sufficient penetration and diffusion of polyalcohol, whereafter the blocks are dried and, thus, the polyalcohol concentrates upon the removal of water. The block surfaces are ground and the outlines are worked to precise measures. Thereafter, the blocks are glued into blanks of board parquet, i.e. fitted between two body layers 4. Attachment to the body layer 4 of a parquet element can be effected by using a resin or wood adhesive 5 (e.g. a polyester resin or a polyvinyl acetate glue). The body 4 can preferably be made of plywood having a thickness of e.g. 9 mm. The body 4 may also include one or a plurality of reinforced plastic layers. The blank is sawn in two parts in the middle of wood blocks 1 and the resulting boards are provided with butments and the sawn surfaces are ground. Following the sawing and grinding, the vertical-grained surface layer 1 has a thickness of e.g. 3,0 - 3,5 mm.

To the surface of a finished wood parquet element is applied some filling resin or varnish which is allowed to impregnate inside wood grains and in interstices therebetween. The impregnation of filling resin is accelerated basically the same way as described above in relation to the impregnation of PEG. Thus, the boards are pre-heated and, upon cooling, they absorb the resin to a sufficient depth inside wood grains and in the interstices therebetween. The employed filling resin or varnish is preferably some inexpensive polyester resin to maintain the parquet manufacturing costs reasonable despite the fact that, due to the porosity of the surface, the required amount of resin will be more than 100 g/m², typically 100 - 300 g/m², preferably 150 - 200 g/m². Thus, the filling resin or varnish impregnates locally to the depth of up to 0,5 mm and over most of the surface area to the depth of more than 0,2 mm. Thus, the thickness of a filling resin or varnish layer 2 varies according to the porosity and absorbing capacity of wood but remains typically within the above range. The process preferably involves the use of a UV-setting polyester resin but also a conventional extra heat activated (accelerated) curing reaction is possible. The layer built by filling resin or varnish 2 improves substantially the wear resistance and hardness of vertical-grained wood. The surface filling layer also provides an extra barrier against the penetration of moisture and at the same time braces the structure against the forces created by the remaining moisture-induced movements.

By virtue of filling layer 2 the consumption of expensive parquet lacquers, such as UV-setting polyurethane lacquers, remains on the same level as or lower than in conventional board parquets, i.e. it is typically 20 - 50 g/m². Thus, the amount of wood-impregnating filling resin or varnish is appr. 4 - 5 times that of a parquet lacquer. The filling resin may also be one of the following alternatives: acrylic resin, epoxy resin, urea formaldehyde and phenolic resin. A clear, colourless polyester resin is preferable as it is capable of well bringing out the inherent hues and natural beauty of wood. If necessary, the filling resin can be admixed with whitening pigments, such as titanium white or resin-soluble colourants.

A method of the invention can also be used for manufacturing high-quality parquet from soft grades of wood. For example, tests have been made with alder to manufacture a vertical-grained wood parquet having about a double hardness and a multiple wear resistance compared with normal oakwood parquet. Also aspen can be used to manufacture a parquet competitive with current grades of parquet in terms of its wear resistance and hardness. The same applies also to the relatives of aspen, e.g. poplar. In fact, one discovery and advantage of the invention relates to the very use of soft grades of wood. Since the compression strength of soft grades of wood in the transverse direction of grains is low, also the cross-grain directed forces, which the grain structure is able to transmit, remain low and this is another reason why the contact-induced movements of parquet remain quite negligible.

An individual parquet element can be made relatively wide (e.g. 278 mm) whereby, when using wood blocks different from each other in terms of colour tones and sizes/shapes, it is possible to create an extensive selection of designs by varying their lay-down patterns. A possibility of using inexpensive timber materials, such as alder and aspen, renders a parquet structure of the invention competitive also in terms of price.

This method can be applied for manufacturing a ready-made parquet or board parquet but it can also be applied as a genuine parquet, which is directly laid down on the floor and corresponds to a traditional block parquet with the blocks glued directly to the floor, ground and varnished with parquet lacquers.

## Claims

1. A parquet structure, wherein the direction of the grains of wood building a parquet surface layer (1) is perpendicular or at an acute angle relative to the level of a parquet surface, **characterized** in that underneath parquet lacquer layers (3) making up the actual surface varnish there is a filling resin or varnish (2) impregnated inside and in the interstices of vertical wood grains, the amount of said varnish being multiple, preferably 4 - 5 times with respect to the amount of said parquet lacquer.

2. A parquet structure as set forth in claim 1, **characterized** in that said filling resin or varnish absorbable in wood (1) is impregnated inside wood to a depth of 0,1 - 0,5 mm and this resin or varnish layer (2) is covered with an actual parquet lacquer layer (3).

3. A parquet structure as set forth in claim 1 or 2, **characterized** in that said filling resin (2) consists of a UV-setting polyester resin and said parquet lacquer (3) consists of a UV-setting urethane lacquer.

4. A parquet structure as set forth in any of claims 1 - 3, **characterized** in that the amount of filling resin or varnish (2) is 4 - 5 times that of parquet lacquer (3) and the filling resin is one of the following resins: polyester resin, acrylic resin, epoxy resin, ureaformaldehyde and phenolic resin.

5. A parquet structure as set forth in any of claims 1 - 4, **characterized** in that the filling resin is admixed with whitening pigments, such as titanium white or resin-soluble colourants.

6. A parquet structure as set forth in any of claims 1 - 5, **characterized** in that the amount of filling resin or varnish is 100 - 300 g/m² and the amount of parquet lacquer (1) is 20 - 50 g/m².

7. A parquet structure as set forth in claim 1 or 2, **characterized** in that the wood blocks forming said surface wood layer (1) are impregnated with a water-soluble polyalcohol, for example polyethylene glycol, which replaces some of the cell-wall water of wood.

8. A method for manufacturing a parquet, said method comprising the following operations:
- laying a parquet body (4) with a surface layer (1) of wood which is made of wood blocks, wherein the direction of wood grains is perpendicular or at an acute angle relative to the level of a parquet surface;
- effecting the smooth grinding of a surface and
- effecting the lacquer finish with a parquet lacquer,
**characterized** in that prior to the lacquer finishing the parquet surface is coated with a filling resin or varnish (2) impregnating inside and in the interstices of vertical wood grains, the amount of said resin being multiple, preferably about 4 - 5 times as compared with the amount of parquet lacquer.

9. A method as set forth in claim 8, **characterized** in that prior to laying the surface wood layer (1) forming wood blocks on said body (4), the wood blocks are impregnated with a water-soluble polyalcohol, e.g. polyethylene glycol, which is allowed to have effect on the wood blocks for replacing some of the cell-wall water therein.

10. A method as set forth in claim 8 or 9, **characterized** in that the amount of filling resin or varnish impregnated in the surface of a finished wood parquet is more than 100 g/m², preferably 150 - 200 g/m² and on top of this is applied some parquet lacquer in the amount of 20 - 50 g/m².

11. A method as set forth in any of claims 8 - 10, **characterized** in that said filling resin or varnish (2) is impregnated inside heated wood during its cooling stage to a depth of 0,2 - 0,5 mm, and after the setting of this resin or varnish layer (2), it is coated by applying an actual parquet lacquer layer (3) which consists of urethane lacquer.

## Patentansprüche

1. Parkettstruktur, bei der die Richtung der Maserungen eines eine Parkett-Oberflächenschicht (1) bildenden Holzes im Verhältnis zur Ebene der Parkettoberfläche rechtwinklig oder in einem spitzen Winkel verläuft,
dadurch gekennzeichnet,
daß unterhalb der den eigentlichen Oberflächenlack bildenden Parkett-Firnisschichten (3) ein Füllharz oder Lack in das Innere und in die Zwischenräume von vertikalen Holzmaserungen einimpregniert ist und daß die Menge des Lackes bezogen auf die Menge des Parkettfirnisses ein Vielfaches, vorzugsweise ein 4 - 5 faches ist.

2. Parkettstruktur nach Anspruch 1,
dadurch gekennzeichnet,
daß das oder der von dem Holz (1) absorbierbare Füllharz oder Lack bis zu einer Tiefe von 0,1 - 0,5 mm in das Holz einimpregniert ist und daß die Harz- oder Lackschicht (2) von der eigentlichen Firnisschicht (3) bedeckt ist.

3. Parkettstruktur nach Anspruch 1 oder 2,
dadurch gekennzeichnet,
daß das Füllharz (2) aus einem UV-setzenden Polyester-Harz und der Parkettfirnis (3) aus einem UV-setzenden Urethan-Firnis besteht.

4. Parkettstruktur nach einem oder mehreren der Ansprüche 1 bis 3,
dadurch gekennzeichnet,
daß die Menge des Füllharzes oder Lackes (2) der 4 - 5 fachen Menge des Parkettfirnisses (3) entspricht und daß das Füllharz eines der folgenden Harze ist: Polyester-Harz, Acryl-Harz, Epoxyd-Harz, Ureaformaldehyd- und Phenol-Harz.

5. Parkettstruktur nach einem oder mehreren der Ansprüche 1 bis 4,
dadurch dekennzeichnet,
daß das Füllharz mit weißen Pigmenten, wie zum Beispiel Titan-Weiß, oder mit harzlöslichen Farbstoffen vermischt ist.

6. Parkettstruktur nach einem oder mehreren der Ansprüche 1 bis 5,
dadurch gekennzeichnet,
daß die Menge des Füllharzes oder Lackes 100 - 300 g/m² und die Menge des Parkettfirnisses (1) 20-50 g/m² beträgt.

7. Parkettstruktur nach Anspruch 1 oder 2,
dadurch gekennzeichnet,
daß die die Oberflächenholzschicht (1) bildenden Holzblöcke mit einem wasserlöslichen Polyalkohol, wie zum Beispiel Polyethylen-Glycol, impregniert sind, das einiges Zellwandwasser des Holzes ersetzt.

8. Verfahren zur Herstellung eines Parketts umfassend die folgenden Arbeitsgänge:
- Belegung eines Parkettkörpers (4) mit einer Oberflächenschicht (1) aus Holz, die aus Holzblöcken hergestellt ist, wobei die Richtung der Holzmaserungen im Verhältnis zur Ebene der Parkettfläche rechtwinklig oder in einem spitzen Winkel verläuft,
- Ausführung eines glatten Oberflächenschliffs und
- Ausführung des Firnisanstrichs mit einem Parkettfirnis,
dadurch gekennzeichnet,
daß die Parkettoberfläche vor dem Firnisanstrich mit einem Füllharz oder Lack (2) beschichtet wird, das oder der ins Innere und in die Zwischenräume der vertikalen Holzmaserungen einimpregniert und daß die Menge des Harzes bezogen auf die Menge des Parkettfirnisses ein Vielfaches, vorzugsweise etwa ein 4 - 5 faches beträgt.

9. Verfahren nach Anspruch 8,
dadurch gekennzeichnet,
daß vor der Auslegung der die Oberflächenholzschicht (1) auf dem Körper (4) bildenden Holzblöcke diese mit einem wasserlöslichen Polyalkohol, wie zum Beispiel Polyethylen-Glycol, impregniert werden, welches imstande ist, auf die Holzblöcke einzuwirken, um einiges darin enthaltenes Zellwandwasser zu ersetzen.

10. Verfahren nach Anspruch 8 oder 9,
dadurch gekennzeichnet,
daß die Menge des in die Oberfläche eines bearbeiteten Holzparketts einimpregnierten Füllharzes oder Lackes mehr als 100 g/m² , vorzugsweise 150 - 200 g/m² beträgt und daß darauf ein Parkettfirnis in der Menge von 20 - 50 g/m² aufgebracht wird.

11. Verfahren nach einem oder mehreren der Ansprüche 8 - 10,
dadurch gekennzeichnet,
daß der Füllharz oder Lack (2) während des Abkühlvorgangs von erhitztem Holz in eine Tiefe von 0,2 - 0,5 mm in das Innere des Holzes einimpregniert wird und daß nach dem Abbinden der Harz- oder Lackschicht (2) diese durch aufbringen einer eigentlichen Parkettlfirnisschicht (3), die aus Urethan-Firnis besteht, beschichtet wird.

## Revendications

1. Structure de parquet, dans laquelle la direction des grains du bois constituant une couche de surface de parquet (1) est perpendiculaire au niveau d'une surface du parquet ou forme un angle aigu par rapport à celui-ci, caractérisée en ce qu'en dessous de couches de laque de parquet (3) constituant le vernis de surface proprement dit se trouve une résine ou un vernis de remplissage (2) imprégnant l'intérieur de grains verticaux du bois et les interstices entre ceux-ci, la quantité dudit vernis étant un multiple, de préférence 4-5 fois par rapport à la quantité de ladite laque de parquet.

2. Structure de parquet selon la revendication 1, caractérisée en ce que ladite résine ou ledit vernis de remplissage que le bois (1) peut absorber imprègne l'intérieur du bois à une profondeur de 0,1-0,5 mm, et cette couche de résine ou de vernis (2) est recouverte d'une couche de laque de parquet (3) proprement dite.

3. Structure de parquet selon la revendication 1 ou 2, caractérisée en ce que ladite résine de remplissage (2) est constituée d'une résine polyester durcissant aux UV, et ladite laque de parquet (3) est constituée d'une laque d'uréthane durcissant aux UV.

4. Structure de parquet selon l'une quelconque des revendications 1-3, caractérisée en ce que la quantité de résine ou de vernis de remplissage (2) vaut 4-5 fois celle de la laque de parquet (3), et la résine de remplissage est une des résines suivantes: résine de polyester, résine acrylique, résine époxy, résine d'uréeformaldéhyde et phénolique.

5. Structure de parquet selon l'une quelconque des revendications 1-4, caractérisée en ce qu'à la résine de remplissage sont mélangés des pigments de blanchissement tels que du blanc de titane ou des colorants solubles dans la résine.

6. Structure de parquet selon l'une quelconque des revendications 1-5, caractérisée en ce que la quantité de résine ou de vernis de remplissage est de 100-300 g/m², et la quantité de laque de parquet (1) est de 20-50 g/m².

7. Structure de parquet selon la revendication 1 ou 2, caractérisée en ce que les blocs de bois formant ladite couche de bois de surface (1) sont imprégnés d'un polyalcool soluble dans l'eau, par exemple de polyéthylèneglycol, qui remplace une partie de l'eau des parois cellulaires du bois.

8. Procédé de fabrication d'un parquet, ledit procédé comportant les opérations ci-dessous:
- pose d'un corps de parquet (4) présentant une couche de surface en bois (1) constituée de blocs de bois, dans laquelle la direction des grains du bois est perpendiculaire au niveau d'une surface de parquet ou forme un angle aigu par rapport à celui-ci;
- exécution d'un ponçage d'une surface, et
- finition à la laque avec une laque de parquet,
caractérisé en ce qu'avant la finition à la laque, la surface de parquet est revêtue d'une résine ou d'un vernis de remplissage (2) imprégnant l'intérieur des grains verticaux du bois et les interstices entre ceux-ci, la quantité de ladite résine constituant un multiple, de préférence environ 4-5 fois comparée à la quantité de la laque de parquet.

9. Procédé selon la revendication 8, caractérisé en ce qu'avant de poser la couche de bois de surface (1) formée de blocs de bois sur ledit corps (4), les blocs de bois sont imprégnés d'un polyalcool soluble dans l'eau, par exemple de polyéthylèneglycol, que l'on laisse agir sur les blocs de bois pour y remplacer une partie de l'eau des parois cellulaires.

10. Procédé selon la revendication 8 ou 9, caractérisé en ce que la quantité de résine ou de vernis de remplissage imprégnant la surface d'un parquet de bois fini est supérieure à 100 g/m², de préférence de 150-200 g/m², et que par dessus celle-ci est appliquée une laque de parquet en quantité de 20-50 g/m².

11. Procédé selon l'une quelconque des revendications 8-10, caractérisé en ce qu'au cours de l'étape de refroidissement du bois chauffé, ladite résine ou ledit vernis de remplissage (2) imprègne l'intérieur du bois jusqu'à une profondeur de 0,2-0,5 mm, et lorsque cette couche de résine ou de vernis (2) a durci, elle est revêtue par application d'une couche de laque de parquet (3) proprement dite, qui est constituée de laque d'uréthane.
